

# UNITED STATES PATENT OFFICE.

CHARLES ALLUISI, OF MONTREAL, CANADA, ASSIGNOR OF ONE-HALF TO  
HORMISDAS CONSTANT, OF SAME PLACE.

## PLASTER COMPOUND.

SPECIFICATION forming part of Letters Patent No. 562,449, dated June 23, 1896.

Application filed April 21, 1896. Serial No. 588,497. (No specimens.) Patented in Canada March 24, 1896, No. 51,742.

*To all whom it may concern:*

Be it known that I, CHARLES ALLUISI, a citizen of the Dominion of Canada, residing at the city of Montreal, in the district of Montreal and Province of Quebec, Canada, have invented certain new and useful Improvements in Plaster Compounds, (for which I have obtained a patent in Canada, No. 51,742, dated March 24, 1896;) and I do hereby declare the following to be a full, clear, and exact description of the invention, such as will enable others skilled in the art to which it appertains to make and use the same.

This invention relates to plaster compound; and it consists in the composition of matter hereinafter fully described and claimed.

This composition consists of the following ingredients, combined in the proportions stated, viz: pure water, one hundred and twenty gallons; asbestos, (crushed,) two thou-

sand pounds; sulfate of lime, six hundred pounds; glue, forty pounds; whitening, two hundred pounds; sulfate of potash, ten pounds. These ingredients are to be thoroughly mingled by agitation.

25

This composition is specially convenient for making plastering and any rosace or capital.

What I claim, and desire to secure by Letters Patent of the United States, is—

The herein-described plaster compound, 30 consisting of pure water, asbestos, sulfate of lime, glue, whitening and sulfate of potash, in the proportions specified.

In testimony whereof I affix my signature in presence of two witnesses.

CHARLES ALLUISI.

Witnesses:

T. C. LABERGE,  
J. A. MARION.

It is hereby certified that the name of the assignee in Letters Patent No. 562,449, granted June 23, 1896, upon the application of Charles Alluisi, of Montreal, Canada, for an improvement in "Plaster Compounds," was erroneously written and printed "Hormisdas Constant," whereas said name should have been written and printed *Hormisdas Constant*; and that the said Letters Patent should be read with this correction therein that the same may conform to the record of the case in the Patent Office.

Signed, countersigned, and sealed this 11th day of August, A. D. 1896.

[SEAL.]

JNO. M. REYNOLDS,  
*Assistant Secretary of the Interior.*

Countersigned:

JOHN S. SEYMOUR,  
*Commissioner of Patents.*